

# United States Patent

[19]

Hori et al.

[11] 3,886,722

[45] June 3, 1975

[54] **PROCESS FOR PRODUCING POLYESTER TEXTURED YARN**

[75] Inventors: **Kikuo Hori; Hidehiko Okada; Masakazu Fujita, all of Matsuyama, Japan**

[73] Assignee: **Teijin Limited, Osaka, Japan**

[22] Filed: **Aug. 13, 1973**

[21] Appl. No.: **387,629**

[30] **Foreign Application Priority Data**

Aug. 17, 1972 Japan ..... 47-81782

[52] **U.S. Cl. .... 57/157 TS**

[51] **Int. Cl. .... D02g 1/00**

[58] **Field of Search..... 57/34 HS, 157 R, 157 S, 57/157 TS, 157 MS, 160**

[56] **References Cited**

UNITED STATES PATENTS

|           |        |                    |             |
|-----------|--------|--------------------|-------------|
| 3,090,997 | 5/1963 | Tin-Yam Au .....   | 57/157 S UX |
| 3,137,991 | 6/1964 | Fairley .....      | 57/160      |
| 3,400,194 | 9/1968 | Boone et al. ..... | 57/157 S X  |

|           |         |                    |            |
|-----------|---------|--------------------|------------|
| 3,481,136 | 12/1969 | Timmons et al..... | 57/157 S X |
| 3,691,750 | 9/1972  | Waters.....        | 57/160 X   |
| 3,780,515 | 12/1973 | Waters.....        | 57/157 R   |

*Primary Examiner—Donald E. Watkins  
Attorney, Agent, or Firm—Sherman & Shalloway*

[57] **ABSTRACT**

A process for producing a polyester textured yarn which comprises drawing and simultaneously false-twisting an undrawn polyester yarn using a draw texturing apparatus equipped with a heat-treating heater and a false twister between feed rollers and draw rollers, wherein the undrawn polyester yarn has a birefringence ( $\Delta n$ ) of 0.01 to 0.05, and the draw ratio (DR) is adjusted to a value expressed by the following equations according to the birefringence of the undrawn polyester yarn

$$-1.8349 \log \Delta n - 1.1376 \quad DR = -2.1789 \log \Delta n - 1.3509$$

and

$$DR = 2.8.$$

**17 Claims, 5 Drawing Figures**



Fig. 1



Fig. 4



Fig. 2





PROCESS FOR PRODUCING POLYESTER  
TEXTURED YARN

This invention relates to a method of producing polyester textured yarns. More specifically, this invention relates to a method of producing textured yarns which comprises drawing an undrawn yarn of a polyester using a draw texturing apparatus including a heat-treating heater and a false twister between feed rollers and draw rollers, and simultaneously false-twisting it to form a textured yarn.

In recent years, a method of producing a textured yarn from an undrawn yarn in a single step has been in use, in which an undrawn yarn of polyester is drawn and simultaneously twisted. Although this method is very efficient as compared with the conventional method in which drawing and twisting are performed separately, there is a defect that because of the occurrence of fluffs, loops, tight spots, dyeing unevenness, etc., textured yarns of fully satisfactory quality cannot be obtained.

It is an object of this invention to provide a draw-texturing process capable of providing textured yarns free from these defects.

We have found that the above object can be achieved by selecting an undrawn yarn of a specific birefringence and a specific draw ratio is selected according to the birefringence of the undrawn yarn.

According to this invention, there is provided a method of producing polyester textured yarns which comprises drawing and simultaneously false twisting an undrawn yarn of a polyester using a draw texturing apparatus equipped with a heat-treating heater and a false twister between feed rollers and draw rollers, wherein the undrawn yarn of polyester has a birefringence ( $\Delta n$ ) of 0.01 to 0.05, and the draw ratio (DR), that is, the ratio of the peripheral speed of the draw rollers and that of the feed rollers, is adjusted to a value which satisfy the following equation according to the birefringence of the undrawn yarn

$$-1.8349 \log \Delta n - 1.1376 \leq DR \leq -2.1789 \log \Delta n - 1.3509$$

$$DR \leq 2.8$$

The "polyester undrawn yarn," as used in the present specification and appended claims, generically denotes "a substantially unoriented multifilament yarn composed of polyethylene terephthalate or a copolymer at least 85 mol % of which are ethylene terephthalate units." The denier, and cross sectional configuration of the multifilament yarn and the addition of an additive thereto, etc. can be selected as desired. For textured yarns having good feel, undrawn yarns having a denier size of 30 to 1,000 denier are especially preferred.

In the present invention, the polyester undrawn yarns having a birefringence ( $\Delta n$ ) of 0.01 to 0.05, preferably 0.01 to 0.025, are used. The birefringence of the undrawn yarn varies according to such factors as the composition, and inherent viscosity of the polyester, the spinning temperature, spinning speed, or the cooling conditions. By controlling these conditions, undrawn yarns having a birefringence of 0.01 to 0.05 can be easily produced.

For example, when polyethylene terephthalate having an inherent viscosity (as measured in  $\sigma$ -chlorophenol at 35°C.) of 0.6 is spun at 300°C. using a conventional spinning apparatus, and wound up at

various rates, the birefringence of the resulting filament changes as shown below.

| Wind-up rates<br>(m/min.) | Birefringence |
|---------------------------|---------------|
| 1000                      | 0.0053        |
| 1500                      | 0.0102        |
| 2000                      | 0.0184        |
| 2700                      | 0.0312        |
| 3000                      | 0.0391        |
| 3500                      | 0.0485        |
| 4000                      | 0.0652        |

If an undrawn yarn of polyester in this invention is less than 0.01, breakage of the yarn frequently occurs at the time of yarn stringing, and the efficiency of the yarn stringing and the productivity become poor. In addition, tight spots tend to occur and the undrawn yarn drastically changes with the passage of time, making it impossible to produce a textured yarn of uniform quality. On the other hand, with an undrawn yarn having a birefringence exceeding 0.05, non-uniformity in the spinning process is remarkable, and this non-uniformity cannot be obviated even by draw texturing techniques, thus making it impossible to give a textured yarn of uniform quality.

In the present invention, it is preferred that an undrawn polyester yarn which has been subjected to aging under the temperature ( $T^{\circ}\text{C}.$ )-time ( $t$  hours) conditions be submitted to a draw texturing process. In this case, a textured yarn having especially reduced occurrence of dyeing unevenness can be obtained.

Aging conditions:

$$\text{where } 20^{\circ}\text{C.} \leq T \leq 30^{\circ}\text{C.}, t_{10}(2.604 - 0.0486T) \leq$$

$$t \leq -211.2T + 6424$$

$$\text{where } 30^{\circ}\text{C.} \leq T \leq 40^{\circ}\text{C.}, t_{10}(2.604 - 0.0486T) \leq$$

$$t \leq t_{10}(3.259 - 0.0526T)$$

An alternative method of obtaining a textured yarn having especially reduced occurrence of dyeing unevenness involves the use of an undrawn polyester yarn whose moisture content is maintained always at not more than 1.0% preferably not more than 0.5%, during the period from the end of spinning until the draw texturing process. Adjustment of the moisture content of the undrawn yarn to such a low value can be easily achieved by treating the undrawn yarn with an oiling agent having a low moisture content or having substantially no moisture content in the spinning step.

FIG. 1 is a side elevation in simplified form of a suitable apparatus for performing the method of the invention;

FIG. 2 is a sectional view illustrating a preferred embodiment of this invention for performing the method of this invention using a modified hot-plate type heater;

FIG. 3 is a graphic representation showing the relation between draw ratio and birefringence;

FIG. 4 is a side elevation illustrating still another embodiment of an apparatus usable in this invention;

FIG. 5 is a graphic representation showing the relationship between yarn parameters of this invention.

FIG. 1 of the accompanying drawings is a side elevation in simplified form of one example of a suitable apparatus for performing the method of this invention. In FIG. 1, the reference numeral 1 shows a package of an undrawn yarn; 2, a tensioner; 3, feed rollers; 4, a heat-treating heater; 5, a false-twisting spindle; 6, draw rollers; and 7, a winder. The undrawn yarn is withdrawn

from the package 1, and fed at a constant speed by the feed rollers 3 via the tensioner 2. After making sliding contact with the heat-treating heater 4, the undrawn yarn passes the false twisting spindle 5 and reaches the draw rollers 6 which rotate at a constant speed faster than the speed of the feed rollers. During this time, the undrawn yarn is drawn at a draw ratio (DR) corresponding to the ratio of peripheral speed between the draw rollers 6 and the feed rollers 3, and the false twists given to the yarn by the false-twisting spindle 5 are heat-set by the heat-treating heater 4. The false twists are detwisted after passage of the yarn through the false twisting spindle 5. The position of the undrawn yarn on the heat-treating heater is fixed by a guide located upwardly of the heater 4 and a guide located downwardly of the heater 4, and the feeding position of the yarn to the false twisting spindle 5 is fixed by a guide located upwardly of the spindle 5. The drawn yarn which has left the draw rollers 6 develops crimps while being wound up by the winder 7 after passing the guide. The draw texturing speed is usually 75 to 600 m/min.

The heat-treating heater is not limited to a hot plate type as shown in FIG. 1, but other known types such as a slit heater or tube heater can be used. Preferably, the temperature of the heat-treating heater is 160° to 210°C. When temperatures within this range are employed, textured yarns having especially good level-dyeability and crimp properties with extremely reduced occurrence of fluffs or tight spots can be obtained.

According to another preferred embodiment of this invention, the surfaces of the feed rollers 3 are maintained at a temperature of 60° to 120°C., and the undrawn yarn is brought into contact with the surfaces for at least 0.05 second. By this procedure, the point of drawing is fixed between the feed rollers 3 and the heat-treating heater 4, and the occurrence of drawing unevenness, dyeing unevenness, yarn breakage, and fluffs, etc., is remarkably reduced.

FIG. 2 of the accompanying drawings is a sectional view for illustrating a preferred embodiment of this invention for performing the method of this invention using a modified hot plate-type heater 4' instead of the hot plate shown in FIG. 1. In FIG. 2, the reference numeral 1 shows an undrawn yarn, and the reference numeral 9 shows one member of a pair of walls arranged in parallel with each other with a slit therebetween in the longitudinal direction of the heater 4'. In this embodiment, the undrawn yarn 1 does not come into contact with the heated surface of the heater from the inlet of the heater to a position apart from it by distance  $l$  mm., but is preheated at a temperature of 60° to 150°C. within the slit space confined by the wall 9. The undrawn yarn is subsequently brought into contact with the heated surface of the heater. The distance  $l$  should satisfy the following equations.

$$l \geq 5$$

and

$$0.03x + 0.2y - 15l \leq 0.3x + 2y + 100$$

wherein  $x$  is the denier size of the undrawn yarn, and  $y$  is the feed rate (m/min) of the undrawn yarn. If the undrawn yarn is heat-treated under these conditions, the point of drawing is fixed between the point of initial contact of the undrawn yarn with the heated surface of the heater and a point 30 mm away from it, and therefore, a textured yarn having especially superior crimp

properties and reduced occurrence of tight spots, dyeing unevenness and fluffs can be obtained.

The rotating speed of the false-twisting spindle 5 is preferably controlled such that the twist multiplier  $\alpha$  expressed by the following equation is within the range of 0.85 and 1.15.

$$\alpha = x \cdot \frac{\sqrt{De}}{32500}$$

wherein  $x$  is the number of false twists (T/M), and  $De$  is the denier of the drawn yarn.

It is essential in the present invention that the ratio of the peripheral speed of the draw rollers 6 to that of the feed rollers 5, that is, the draw ratio (DR), be adjusted to a value expressed by the following equations according to the birefringence ( $\Delta n$ ) of the undrawn yarn, for example within the range of 2.2 to 2.8.  $-1.8349 \log \Delta n - 1.1376 \leq DR \leq -2.1789 \log \Delta n - 1.3509$   $DR \leq 2.8$

FIG. 3 of the accompanying drawings is a graphic representation showing the relation between the draw ratio and the birefringence. In performing the method of this invention, the draw ratio and birefringence values within the hatched area in FIG. 3 should be selected. If the draw ratio is lower than this range, the undrawn yarn melt-adheres onto the heat-treating heater, and yarn stringing is difficult. Moreover, the level-dyeability becomes poor, and the tenacity is reduced. On the other hand, if the draw ratio is higher than the range specified above, fluffs and loops tend to occur, and the crimp characteristics of the yarn become poor. Furthermore, when the draw ratio becomes too high, the tenacity of the yarn rather decreases.

As is clear from FIG. 3, the draw ratio employed in the method of this invention is considerably lower than those employed in usual drawing processes. It is surprising that in spite of the use of such low draw ratios, the method of this invention makes it possible to give a texture yarn having no fluffs or loops and having superior level-dyeability, mechanical properties and crimp characteristics.

Another embodiment is possible in this invention in which at least 2 yarn guides are provided between the false twister and the draw rollers to bend the yarn at a certain angle, and the total sum of the bended angles caused by these guides is adjusted to 30° to 270°C., preferably 30° to 150°.

FIG. 4 is a side elevation illustrating this embodiment of this invention. The reference numeral shows a false twisting spindle, the reference numerals 8, 8' and 8'' show yarn guides, and the reference numeral 10 designates draw rollers. Of course, the draw rollers 10 may be replaced by the draw rollers 6 shown in FIG. 1. In this embodiment also, it goes without saying that package 1, tensioner 2, feed rollers 3, heat-treating heater 4, winder 7, etc. must be arranged as shown in FIG. 1.

According to this embodiment, as shown in FIG. 4, at least two yarn guides 8, 8', 8'' ... are provided between the false twisting spindle 5 and the draw rollers 10, and the total sum of the bended angles  $\alpha_1, \alpha_2, \alpha_3, \dots$  ( $\Sigma \alpha$ ) is adjusted to 30° to 270°, preferably 30° to 150°. This total sum of the bended angles is very important for detwisting the false twists completely and exhibiting the crimp characteristics fully. If the total sum is less than 30°, the false twists are not sufficiently detwisted, and tight spots occur partly in the lengthwise

direction of the yarn. On the other hand, if the total sum exceeds 270°, resistance caused by the guides becomes excessive, and fluffs occur. Furthermore, the crimp characteristics become poor. However, if the total sum ( $\Sigma\alpha$ ) is within the range specified in this invention, the false twists are completely detwisted, and the crimp characteristics are improved and the occurrence of ballooning is very much reduced. Furthermore, the number of the yarn guides is also of importance. If it is only one, uniform detwisting can not be performed even if the bended angle of the yarn is adjusted to more than 30°. In order to give a bended angle of more than 30° using one guide, the guide must be provided at a position greatly deviated from the center of the false twisting spindle. However, if it is disposed in such a way, the yarn comes into contact with the edge of the spindle and excessive load is exerted on the yarn, which in turn becomes a cause of fluffs and poor crimps. Accordingly, it is necessary to provide at least two yarn guides.

False twisting can also be performed using known false-twisting means, for example, by applying friction or by a swirling flow of fluid. In the example shown in FIG. 4, the bended direction of the yarn is at right angles to the axial direction of the draw rollers, but may be in the parallel direction to the axial direction of the draw rollers. Further, bendings in both directions may be combined as desired.

The shape and dimension of the yarn guide are not particularly restricted, but preferably, the guide nearest the false twister is an annular guide, and the other guides are rod-like guides. Further, the guides may be either fixed guides or rotating guides. The surface of the guides may either be smooth or embossed. However, especially by using fixed guides with smooth surfaces of not more than 1S, the effect of preventing tight spot is remarkable. In addition, by the contacting effect of the guides, the crimp characteristics of the yarn are improved to a great degree. The material of the guides may be those conventionally used, for example, sapphire, titanium porcelain, alumina porcelain, or chrome-plated metals.

According to another embodiment of this invention, the process is controlled so that the yarn is made to run in air at room temperature for 0.13 to 0.3 second between the heat-treating heater and the false twister. This makes it possible to obtain a textured yarn having high degrees of crimp and crimp fastness and reduced tight spot.

According to still another embodiment of this invention, a second heat-treating heater (not shown) is provided following the draw rollers 6 or 10, and enables the draw textured yarn from the draw rolls to be additionally heat-treated at a temperature of 160° to 250°C. while allowing a shrinkage of not more than 50% or while maintaining it at constant length. Thus, the control of the degree of crimping and the improvement of dimensional stability against heat are possible.

The textured yarns produced by the method of this invention are almost free from fluffs, loops and tight spots, and have superior crimp characteristics and mechanical properties and also good level-dyeability. These textured yarns have the advantage that the amount of dye exhaustion does not change even when the temperature of the heat-treating heater fluctuates between 160° and 210°C.

FIG. 5 is a graphic representation showing the relation between the degree of dye exhaustion and the temperature of the heat-treating heater with respect to the texture yarn obtained in the present invention and an ordinary texture yarn. Curve A in this FIG. refers to the textured yarn obtained in this invention, and curve B, to the conventional texture yarn. As is clear from this Figure, with the texture yarn (A) in accordance with this invention, there is scarcely any change in the degree of dye exhaustion when the temperature of the heat-treating heater is within the range of 160° to 210°C. However, with the conventional texture yarn (B), the degree of dye exhaustion changes with the temperatures of the heat-treating heater. Thus, even a slight fluctuation in the temperature of the heater results in dyeing unevenness.

The degree of dye exhaustion denotes the grade of the depth of color observed by the naked eye with a textured yarn which has been dyed by dipping it for 90 minutes in a boiling dye bath containing 2% of Eastman Polyester Blue GLF (CI DISPERSE BLUE 27). Larger numerical values show deeper color.

In the performance of the present invention, various auxiliary means can be employed at the time of initiating the operation or at the time of continuous operation.

Examples of the auxiliary means at the time of initiating the operation are:

1. A method wherein without bringing the yarn into contact with the heat-treating heater, the operation is started using a twist multiplier 50 to 85% of that in normal operation, and then the yarn is brought into contact with the heat-treating heater.

2. A method wherein the operation is started at a draw texturing speed expressed by the equation.

$$5 \leq V \leq 80 - \left( \frac{D_e}{5} \right)$$

wherein V is the draw texturing speed, and yarn stringing is performed, and then the draw texturing speed is raised to a predetermined value.

3. A method wherein at the time of initiating the operation, yarn stringing is performed while the undrawn yarn is maintained so as not to come close to the surface of the heat-treating heater, and then the draw texturing of the yarn is started while passing the yarn through a zone near the surface of the heat-treating heater which zone is held at 50° to 130°C., and then the yarn is brought into contact with the heat-treating heater.

If such auxiliary means are applied, the breakage of yarn at the time of initiating the draw texturing process and at the time of contacting the yarn with the heat-treating heater can be substantially prevented, and therefore, the efficiency of the yarn stringing operation and the working efficiency of the draw texturing apparatus are drastically increased.

Examples of the auxiliary means at the time of continuous operation are:

1. A method wherein the end of the undrawn yarn on the package and the forward end of the undrawn yarn on the package are cold drawn and tied before the package of the undrawn yarn being processed becomes empty.

2. A method wherein at the time of exchange of undrawn yarn, vehicles carrying undrawn yarn package

are arranged in a plurality of rows, and the transfer of the yarn is performed between two packages facing each other on the vehicles.

If such auxiliary means are applied, it is possible to perform the draw texturing process of this invention continuously.

The following Examples illustrate the present invention.

The measurement values in the Examples were obtained by the following methods.

#### 1. Loops and Fluffs

The number of fluffs and loops appearing on both end surfaces of 2.5 Kg of a square end cheese (wind-up width 150 m).

#### 2. Tight spot

The number of un-twisted portions (portions remaining alternately twisted in the yarn without detwisting as a result of heat-fusing of filaments to each other) per 10 m of the processed yarn.

#### 3. Degree of total crimp (TC)

An initial load (2 mg/d) and a heavy load (0.2 g/d) were exerted at the same time on a processed yarn of a constant length, and after a lapse of 1 minute, the length of the sample yarn was measured and designated  $l_0$ . Then, only the heavy load was removed, and the yarn was boiled in boiling water for 20 minutes and allowed to dry spontaneously for 24 hours in a free condition. Then, the initial load and the heavy load were exerted on the yarn at the same time, and after a lapse of 1 minute, the length of the sample yarn was measured, and made  $l_1$ . Then, after removing only the heavy load, and after a lapse of 1 minute, the length of the sample was measured and made  $l_2$ . TC is expressed by the following equation.

$$TC = \frac{l_1 - l_2}{l_0} \times 100\%$$

#### 4. Dyeing unevenness

The dyeing used in the dye exhaustion degree test mentioned above was observed by the naked eye, and evaluated on a scale of 5 to 0 as below.

- 5: no dyeing unevenness
- 4: slight dyeing unevenness
- 3: Dyeing unevenness occurred
- 2: Considerable dyeing unevenness
- 1: Great dyeing unevenness
- 0: Great difference in the depth of the color

#### 5. Crimp fastness

A load was exerted on a polyester textured yarn, and the yarn was continuously stretched, and the elongation of the yarn at disappearance of the crimps and its elongation at break were measured. The crimp fastness was calculated by the following equation.

$$\text{Crimp fastness} = \frac{\text{Elongation at the disappearance of crimps}}{\text{Elongation at break}} \times 100 (\%)$$

#### 6. Moisture content

About 20 g of the undrawn yarn located 5 mm outwardly of the surface of the undrawn yarn bobbin and at the central part with respect to the axial direction of the bobbin (that is, the undrawn yarn present in the innermost layer of the package which is not at all exposed to the outer atmosphere) was quickly sampled. The resulting sample was completely dried, and placed in a bottle of a known weight ( $W_0$  g), and the bottle was sealed with a lid. The bottle was then precisely weighed, and the weight was  $W_{1g}$ . The lid was removed, and the bottle was placed in a hot air dried held at a temperature of  $105^\circ \pm 2^\circ\text{C}$ . After drying for 3 hours, the bottle was sealed with the lid and again precisely weighed. The weight was  $W_{2g}$ . The moisture content (%) was calculated as follows:

$$\text{Moisture content} = \frac{W_1 - W_2}{W_2 - W_0} \times 100 (\%)$$

#### 7. Different in dye exhaustion

A standard sample was a texture yarn which was obtained by subjecting an as-spun undrawn yarn to draw texturing within 8 hours. The standard sample and a sample to be measured were knitted side by side, and the knitted fabric obtained was dyed in the same was as the dye exhaustion degree test mentioned above. The difference in dye exhaustion between the measuring sample and the standard sample was evaluated on the resulting dyeings by the naked eye on the scale shown below. The dye exhaustion difference shows an average value of the dye exhaustion difference for 10 samples of the same level.

- 0: Not discriminatable
- +0.5: Slight difference
- +1.0: Difference fully observed
- +1.5: When the yarn having a dye exhaustion difference of 1.0 was assumed to be a standard sample, there is a slight difference
- +2.0: A slight difference observed in the same way as above using a yarn having a dye exhaustion difference of 1.5

The plus symbol means that the sample was dyed deeper than the standard sample, and the minus symbol shows that it was dyed in lighter color than the standard sample.

#### EXAMPLE 1

Undrawn yarns of polyethylene terephthalate having various birefringence values (210 denier/36 filaments) were subjected to draw texturing using the apparatus shown in FIG. 1 under the following conditions.

|                                         |                        |
|-----------------------------------------|------------------------|
| Temperature of the heat-treating heater | 180°C                  |
| Rotating speed of spindle               | $30.1 \times 10^4$ rpm |
| Twist multiplier                        | 1.0                    |
| Draw ratio (DR)                         | 3.14 to 1.30           |
| Draw texturing speed                    | 75.8 to 115.5 m/min.   |

The results are shown in Table 1 below.

Table 1

| Run No. | Undrawn $\Delta n$ | DR   | Draw texturing speed (m/min.) | Yarn stringing      | Loops and fluffs per 25 kg | Tight spots per 10 m | TC (%) | Dyeing unevenness | Overall evaluation |
|---------|--------------------|------|-------------------------------|---------------------|----------------------------|----------------------|--------|-------------------|--------------------|
| 1-1     | 0.0060             | 3.14 | 75.8                          | Frequent yarn break | 23                         | 3-5                  | 32.6   | 3.5               | Poor               |
| 1-2     | 0.0106             | 2.78 | 80.0                          | Good                | 0-2                        | 0-1                  | 34.3   | 4.5               | Good               |
| 1-3     | 0.0184             | 2.30 | 88.5                          | "                   | 0                          | 0                    | 33.7   | 4.5               | Excellent          |
| 1-4     | 0.0278             | 2.00 | 94.9                          | "                   | 0                          | 0                    | 35.1   | 4.5               | "                  |
| 1-5     | 0.0387             | 1.70 | 102.9                         | "                   | 0                          | 0                    | 32.5   | 4.5               | "                  |
| 1-6     | 0.0485             | 1.50 | 109.6                         | "                   | 0                          | 0                    | 34.1   | 4.5               | "                  |
| 1-7     | 0.0552             | 1.35 | 115.5                         | "                   | 0-3                        | 0                    | 32.3   | 3.0               | Fair               |

## EXAMPLE 2

An undrawn polyethylene terephthalate yarn (302 denier/48 fil) having a birefringence of 0.0226 was subjected to draw texturing using an apparatus shown in FIG. 1, under the following conditions.

|                                         |                        |
|-----------------------------------------|------------------------|
| Temperature of the heat-treating heater | 180°C.                 |
| Rotating speed of the spindle           | $30.1 \times 10^4$ r/m |
| Twist multiplier                        | 1.05                   |
| DR                                      | 1.8 to 2.4             |
| Draw texturing speed                    | 114 to 99 m/min.       |

The results are shown in Table 2 below.

Table 2

| Run No. | DR  | Yarn stringing      | Loops and fluffs | Tight spots per 10 m | Tenacity (g/d) | Elongation (%) | TC (%) | Dyeing unevenness | Overall evaluation |
|---------|-----|---------------------|------------------|----------------------|----------------|----------------|--------|-------------------|--------------------|
| 2-1     | 1.8 | Frequent yarn break | 4                | 8                    | 3.17           | 29.2           | 34.7   | 2.5               | Poor               |
| 2-2     | 1.9 | Good                | 1                | 1                    | 3.68           | 26.8           | 33.0   | 4.0               | Good               |
| 2-3     | 2.0 | "                   | 0                | 0                    | 3.72           | 25.3           | 32.8   | 4.5               | Excellent          |
| 2-4     | 2.1 | "                   | 0                | 1                    | 3.82           | 23.6           | 32.5   | 4.2               | "                  |
| 2-5     | 2.2 | "                   | 1                | 0                    | 3.65           | 20.1           | 31.9   | 4.0               | Good               |
| 2-6     | 2.3 | "                   | 15               | 0                    | 3.24           | 18.5           | 30.4   | 3.5               | Poor               |
| 2-7     | 2.4 | "                   | 28               | 2                    | 3.06           | 16.0           | 26.6   | 3.0               | "                  |

## EXAMPLE 3

A polyethylene terephthalate undrawn yarn (366 denier/30 filaments) having a birefringence of 0.0178 was subjected to draw texturing under the conditions shown in Table 3, using two types of apparatus. The physical properties of the resulting texture yarns were compared. The results are shown in Table 1.

Table 3

| Run No.                                                        | Apparatus used     | Figure 1           | 3-1 | 3-2 |
|----------------------------------------------------------------|--------------------|--------------------|-----|-----|
| Processing conditions                                          |                    |                    |     |     |
| Temperature of the drawn pin                                   | —                  | 90°C.              |     |     |
| Temperature of the hot plate of the heat-treating heater (°C.) | 200                | 210                | 60  |     |
| Rotating speed (rpm) of the spindle                            | $41.5 \times 10^4$ | $41.5 \times 10^4$ |     |     |
| Twist multiplier                                               | 0.98               | 0.98               |     |     |
| DR                                                             | 2.38               | 2.6                |     |     |
| Draw texturing speed (m/min.)                                  | 161.6              | 154.5              |     |     |
| Physical properties of the yarn                                |                    |                    |     |     |
| Loops and fluffs per 2.5 kg                                    | 0 to 3             | 5 to 15            |     |     |
| TC (%)                                                         | 34                 | 30                 |     |     |
| Torque (T/25 cm)                                               | 20                 | 42                 |     |     |
| Knittability                                                   | Good               | With some problem  |     |     |

15

An undrawn yarn (240 denier/24 filaments) of polyethylene terephthalate having an intrinsic viscosity of 0.0152 and a birefringence of 0.62 (containing 5 mol % of isophthalate) was subjected to draw texturing under the following conditions.

20

|                                         |                        |
|-----------------------------------------|------------------------|
| Temperature of the heat-treating heater | 175°C.                 |
| Rotating speed of the spindle           | $40.2 \times 10^4$ rpm |
| Twist multiplier                        | 0.96                   |
| DR                                      | 2.4                    |

25

## EXAMPLE 4

An undrawn yarn (240 denier/24 filaments) of polyethylene terephthalate having an intrinsic viscosity of 0.0152 and a birefringence of 0.62 (containing 5 mol % of isophthalate) was subjected to draw texturing under the following conditions.

30

|                                         |                        |
|-----------------------------------------|------------------------|
| Temperature of the heat-treating heater | 175°C.                 |
| Rotating speed of the spindle           | $40.2 \times 10^4$ rpm |
| Twist multiplier                        | 0.96                   |
| DR                                      | 2.4                    |

35

The resulting texture yarn was free from fluffs, loops, and tight spots, and exhibited good crimpability with a TC of 32.5 %. When this yarn was dyed in blue color, the color was brilliant, and the yarn had good feel.

40

## EXAMPLE 5

Three polyester undrawn yarns (A, B and C) shown in Table 4 were each subjected to draw texturing under the conditions shown in Table 4 and varying the bended angles of the yarn using an apparatus as shown in FIG. 4 which included 1 to 3 guides between the false twisting spindle and draw rollers. The angle of pulling out the yarn from the spindle was adjusted to 20° in all cases. The results are shown in Table 5. In Table 5, Runs Nos. 7, 8, 9, 12, 13 and 14 are examples of the present invention and the others are for comparative purposes.

45

| Undrawn yarn                  | A                | B                | C                |
|-------------------------------|------------------|------------------|------------------|
| Spinning speed (m/min.)       | 1000             | 1100             | 1500             |
| Denier (d/fil)                | 53(d/48f)        | 340d/24f         | 210d/15f         |
| $\Delta n$                    | 0.0054           | 0.0063           | 0.0104           |
| Processing conditions         |                  |                  |                  |
| Twist multiplier (T/M)        | 2500             | 3000             | 3500             |
| Rotating speed of the spindle | $40 \times 10^4$ | $40 \times 10^4$ | $40 \times 10^4$ |
| DR                            | 3.13             | 3.10             | 2.7              |
| Heater temperature            | 190°C            | 180°C            | 170°C            |

50

## Table 4

Table 5

| Run No. | Number of guides | Undrawn yarn             |                          |                          | A              |             | B                |             | C                |             |
|---------|------------------|--------------------------|--------------------------|--------------------------|----------------|-------------|------------------|-------------|------------------|-------------|
|         |                  | <sup>*4</sup> $\alpha_1$ | <sup>*4</sup> $\alpha_2$ | <sup>*4</sup> $\alpha_3$ | $\Sigma\alpha$ | Tight spots | Loops and fluffs | Tight spots | Loops and fluffs | Tight spots |
| 5-1     | 0                | —                        | —                        | —                        | 0°             | 30          | 30               | 32          | 1                | 37          |
| 5-2     | 10               | —                        | —                        | —                        | 10°            | 27          | 13               | 16          | 0                | 29          |
| 5-3     | 1                | 24                       | —                        | —                        | 24°            | 11          | 5                | 9           | 0                | 25          |
|         |                  | 35                       | —                        | —                        | 35°            | 4           | 15               | 3           | 12               | 3           |
|         |                  | 45                       | —                        | —                        | 45°            | 5           | 40               | 10          | 38               | 6           |
| 5-6     | 8.5              | 9.0                      | —                        | —                        | 17.5°          | 24          | 5                | 6           | 0                | 14          |
| 5-7     | 3                | 27                       | —                        | —                        | 30°            | 2           | 0                | 2           | 0                | 2           |
| 5-8     | 2                | 25                       | 47                       | —                        | 72°            | 1           | 1                | 0           | 1                | 0           |
|         |                  | 52                       | 78.5                     | —                        | 130.5°         | 0           | 1                | 0           | 1                | 0           |
|         |                  | 145                      | 145                      | —                        | 290°           | 2           | 25               | 0           | 18               | 1           |
| 5-10    | —                | —                        | —                        | —                        | —              | —           | —                | —           | —                | 10          |
| 5-11    | 5.5              | 4                        | 15                       | 24.5°                    | 3              | 0           | 13               | 0           | 18               | 0           |
| 5-12    | 5                | 5.5                      | 25.7                     | 36.2°                    | 0              | 0           | 0                | 0           | 0                | 0           |
| 5-13    | 3                | 5.5                      | 43                       | 136.5                    | 185°           | 0           | 3                | 0           | 2                | 0           |
|         |                  | 32                       | 133                      | 102                      | 267°           | 1           | 0                | 0           | 2                | 0           |
|         |                  | 58                       | 140                      | 94                       | 292°           | 5           | 9                | 0           | 15               | 0           |
| 5-15    | —                | —                        | —                        | —                        | —              | —           | —                | —           | —                | 6           |

Note:

\*1: Using only guide 8 shown in FIG. 4.

\*2: Using guides 8 and 8' shown in FIG. 4.

\*3: Using guides 8, 8' and 8'' shown in FIG. 4.

\*4: The bended angle shown in FIG. 4.

## EXAMPLE 6

25

An undrawn yarn (345 denier/30 fil, birefringence 0.013) of polyethylene terephthalate having an intrinsic viscosity of 0.632 as measured in o-chlorophenol at 35°C. was subjected to draw texturing using the apparatus of FIG. 1 under the conditions shown in Table 6.

Example 6 was repeated except that the surface temperature of the feed rollers was adjusted to 90°C. and the time of contact between the undrawn yarn and the feed rollers was varied. The results are shown in Table 7.

Table 7

| Run No. | Contact time (seconds) | Tenacity (g/d) | Elongation (%) | TC (%) | Fluffs | Tight spots | Dyeing unevenness |
|---------|------------------------|----------------|----------------|--------|--------|-------------|-------------------|
| 7-1     | 0.03                   | 3.62           | 33.4           | 12.5   | 3      | 15          | 4.0               |
| 7-2     | 0.06                   | 3.95           | 35.5           | 13.9   | 0      | 0           | 4.5               |
| 7-3     | 0.10                   | 4.11           | 34.3           | 14.3   | 0      | 0           | 4.5               |

The yarn obtained was heat-treated at 200°C. while allowing shrinkage of 14.8 %, and then wound up. The results are shown in Table 6.

40

## EXAMPLE 8

Polyethylene terephthalate chips having an intrinsic viscosity of 0.645 were spun at 291°C. and taken up at a rate of 2,000 m/min. to form an undrawn yarn (355 denier/30 fil) having birefringence of 0.0145. In this spinning process, an oil of the following formulation was applied to the yarn by an oiling roller to an oil pick-up of 1 %. The undrawn yarn was wound up, and allowed to stand for 3 months in an atmosphere held at 40°C., and then subjected to draw texturing under the following conditions.

|                                                           |              |
|-----------------------------------------------------------|--------------|
| Temperature of the surface of the feed rollers            | 50 to 130°C. |
| Time of contact of the undrawn yarn with the feed rollers | 0.06 second  |
| Temperature of the heat-treating heater                   | 195°C.       |
| Twist multiplier                                          | 0.98         |
| Draw ratio                                                | 2.452        |
| Draw texturing speed                                      | 185 m/min.   |

55

Table 6

| Run No. | Temperature of feed rollers (°C) | Tenacity (g/d) | Elongation (%) | T. C. (%) | Fluffs | Tight spots per 10 m | Dyeing unevenness |
|---------|----------------------------------|----------------|----------------|-----------|--------|----------------------|-------------------|
| 6-1     | 55                               | 3.68           | 32.4           | 12.3      | 12     | 36                   | 4.0               |
| 6-2     | 65                               | 3.72           | 34.1           | 12.1      | 2      | 3                    | 4.5               |
| 6-3     | 80                               | 3.93           | 35.7           | 13.8      | 0      | 0                    | 4.5               |
| 6-4     | 100                              | 4.05           | 35.1           | 14.0      | 0      | 0                    | 4.5               |
| 6-5     | 115                              | 3.85           | 34.8           | 14.1      | 1      | 0                    | 4.0               |
| 6-6     | 125                              | 3.24           | 31.3           | 11.6      | 16     | 7                    | 3.0               |

| Formulation of Oil A                        |                |
|---------------------------------------------|----------------|
| Mineral oil                                 | 80 % by weight |
| Ethylene oxide-added<br>oleyl alcohol       | 10 % by weight |
| Octyl phosphonic acid<br>amine              | 40 % by weight |
| Oleic acid tri-<br>ethanolamine             | 6 % by weight  |
| Draw texturing conditions                   |                |
| Draw ratio                                  | 2.3            |
| Temperature of the heat-<br>treating heater | 190°C.         |
| Number of twists                            | 2600 T/M       |
| Processing speed                            | 200 m/min.     |

The results are shown in Table 8.

Table 8

| Run No. | State of oil          | Moisture content immediately after spinning (%) | Moisture content (%) after allowing to stand for 3 months at 40°C. | Dye exhaustion difference | Dyeing unevenness |
|---------|-----------------------|-------------------------------------------------|--------------------------------------------------------------------|---------------------------|-------------------|
| 8-1     | 10 % aqueous emulsion | 3.5                                             | 2.5                                                                | + 4                       | 2.0               |
| 8-2     | 6 % aqueous emulsion  | 1.4                                             | 1.1                                                                | + 2                       | 2.5               |
| 8-3     | 20 % aqueous emulsion | 0.8                                             | 0.7                                                                | + 0.3                     | 4.5               |
| 8-4     | Straight oil          | 0                                               | 0.2                                                                | + 0.3                     | 4.5               |
| 8-5     | * 2-stage oiling      | 0.5                                             | 0.5                                                                | + 0.5                     | 4.5               |

\* 2-stage oiling: first stage = 1 % aqueous solution of sodium diethyl sulfosuccinate  
second stage = straight oil

EXAMPLE 9

Polyethylene terephthalate having an intrinsic viscosity of 0.645 as measured in o-chlorophenol at 35°C. was spun at 292°C. and taken up at a speed of 1,7800 m/min. to form an undrawn yarn having a 1,800 of 0.0135 and a denier of 360 denier per 30 filaments.

The undrawn yarn was subjected to draw texturing using an apparatus of the type shown in FIG. 1 except that the false-twisting spindle and the draw rollers were replaced by those shown in FIG. 4, and a second heat-treating heater was equipped, under the following conditions. At this time, the time during which the yarn ran between the outlet of the first heat-treating heater and the false twisting spindle and the total sum ( $\alpha_1 + \alpha_2$ ) of the yarn bended angles were changed. The results are shown in Table 9.

|                                                |            |
|------------------------------------------------|------------|
| Draw ratio                                     | 2.452      |
| Temperature of the first heat-treating heater  | 210°C.     |
| Temperature of the second heat-treating heater | 205°C.     |
| Number of twists                               | 2590       |
| Draw texturing speed                           | 200 m/min. |

Table 9

| Run No. | Time of yarn travel (seconds) | Yarn bended angle ( $\alpha_1 + \alpha_2$ ) | Tenacity (g/d) | Elongation (%) | Degree of crimps (%) | Crimp fastness (%) | Tight spots per 20 m | Fluffs |
|---------|-------------------------------|---------------------------------------------|----------------|----------------|----------------------|--------------------|----------------------|--------|
| 9-1     | 0.11                          | 40°                                         | 3.4            | 29.6           | 11.0                 | 65                 | 26                   | 24     |
| 9-2     | 0.18                          | 40°                                         | 3.6            | 32.4           | 12.7                 | 92                 | 0.5                  | 0.5    |
| 9-3     | 0.27                          | 40°                                         | 3.6            | 31.5           | 13.0                 | 93                 | 0.8                  | 0.7    |
| 9-4     | 0.36                          | 40°                                         | 3.7            | 32.8           | 10.1                 | 80                 | 4.5                  | 18.0   |
| 9-5     | 0.27                          | 20°                                         | 3.6            | 32.3           | 11.8                 | 87                 | 2.0                  | 0.7    |
| 9-6     | 0.23                          | 65°                                         | 3.5            | 33.6           | 12.6                 | 93                 | 0.2                  | 1.0    |
| 9-7     | 0.27                          | 90°                                         | 3.3            | 32.7           | 13.1                 | 92                 | 0.1                  | 1.3    |
| 9-8     | 0.27                          | 360°                                        | 2.8            | 25.4           | 10.3                 | 70                 | 0.2                  | 3.4    |

Table 10

| Run No. | Temperature of the atmosphere in the aging chamber (°C) | Aging time (hours) |
|---------|---------------------------------------------------------|--------------------|
| 10-1    | 10                                                      | 24                 |
| 10-2    | 26                                                      | 28                 |
| 10-3    | 35                                                      | 12                 |
| 10-4    | 50                                                      | 15                 |
| 10-5    | 26                                                      | 24                 |
| 10-6    | 26                                                      | 36                 |
| 10-7    | 26                                                      | 72                 |
| 10-8    | 26                                                      | 600                |

After aging, the undrawn yarn package was transported to a drawing and false-twisting factory remote from the spinning factory. The time which elapsed from the end of aging to the initiation of drawing and false-twisting was about 20 hours, and the temperature during transportation was 24° to 29°C.

The drawing and false-twisting was performed under the following conditions in a chamber maintained at a temperature of 27°C ± 2°C and a relative humidity of 65 ± 5 %.

|                                                |                 |
|------------------------------------------------|-----------------|
| Draw ratio (DR)                                | 2.45            |
| Temperature of the first heater (hot plate)    | 195°C.          |
| Speed of drawing and false-twisting            | 182 meters/min. |
| Number of false twists                         | 2590 T/M        |
| Temperature of the second heater (slit heater) | 205°C.          |
| Shrinkage on the second heater                 | 14.8%           |

10

The properties of the resulting polyester textured yarns are shown in Table 11.

Table 11

| Run No. | Tenacity (g/d) | Elongation (%) | Dyeing difference | Dyeing unevenness (grade) | Fluffs (%) | Tight spots per 20 m | Processability (times) |
|---------|----------------|----------------|-------------------|---------------------------|------------|----------------------|------------------------|
| 10-1    | 3.7            | 31.5           | + 0.8             | 4.0                       | 12.0       | 36                   | 30                     |
| 10-2    | 3.6            | 32.8           | + 0.2             | 4.5                       | 1.5        | 2                    | 12                     |
| 10-3    | 3.6            | 32.5           | + 0.2             | 4.5                       | 1.3        | 17                   | 11                     |
| 10-4    | 3.1            | 29.4           | + 3.5             | 2.0                       | 48.0       | 18                   | 96                     |
| 10-5    | 3.6            | 33.0           | + 0.3             | 4.5                       | 1.8        | 1.5                  | 10                     |
| 10-6    | 3.5            | 32.5           | + 0.2             | 4.5                       | 2.0        | 2.0                  | 8                      |
| 10-7    | 3.6            | 33.2           | + 0.2             | 4.5                       | 1.5        | 1.0                  | 13                     |
| 10-8    | 3.6            | 31.9           | + 0.3             | 4.5                       | 2.3        | 0.8                  | 12                     |

The dyeing difference shown in the above table was measured in accordance with the following method.

A standard sample was prepared by processing an undrawn yarn immediately after arrival at the factory. An undrawn yarn in the same lot as the sample was processed 5 days after arrival at the factory to form a measuring sample. The standard sample and the measuring sample were knitted side by side to form a sample. The resulting sample was dyed by dipping in a dye bath containing 2 %, based on the weight of the sample, of CI DISPERSE BLUE 27 at 100°C. for 60 minutes with the goods-to-liquor ratio being maintained at 1 : 100, followed by washing with water and drying. After drying, the degree of the difference in dye exhaustion between the standard sample and the measuring sample was evaluated by the naked eye on the same scale as described before the Examples.

What we claim is:

1. A process for producing a polyester textured yarn which comprises drawing and simultaneously false-twisting an undrawn polyester yarn using a draw texturing apparatus equipped with a heat-treating heater and a false twister between feed rollers and draw rollers, wherein the undrawn polyester yarn has a birefringence ( $\Delta n$ ) of 0.01 to 0.05, and the draw ratio (DR) is adjusted to a value expressed by the following equations according to the birefringence of the undrawn polyester yarn

$$-1.8349 \log \Delta n - 1.1376 \leq DR \leq -2.1789 \log \Delta n - 1.3509$$

and

$$DR \leq 2.8.$$

2. The process of claim 1 wherein the undrawn yarn has a birefringence of 0.01 to 0.025.

3. The process of claim 1 wherein the undrawn yarn is one which has been aged under the temperature (T°C)-time (t hours) conditions expressed by the following equations

$${}_{10}(2.604 - 0.0486T) \leq t \leq -211.2T + 6424 \quad (\text{where } 20^\circ\text{C} \leq T \leq 30^\circ\text{C.})$$

or

$${}_{10}(2.604 - 0.0486T) \leq t \leq {}_{10}(3.259 - 0.0526T) \quad (\text{where } 30^\circ\text{C} \leq T \leq 40^\circ\text{C.})$$

4. The process of claim 1 wherein the undrawn yarn is one whose moisture content is maintained always at not more than 1.0 % by weight from the end of spinning to the initiation of draw texturing.

5. The process of claim 1 wherein the undrawn yarn is brought into contact with the surfaces of feed rollers heated at 60° - 120°C. for at least 0.05 second.

6. The process of claim 1 wherein the heat-treating heater is heated to from 160° to 210°C.

7. The process of claim 1 wherein the process is carried out while maintaining a twist multiplier expressed by the following equation

$$\alpha = x \cdot \frac{\sqrt{De}}{32500}$$

wherein  $x$  is the number of false twists (T/M), and  $De$  is the denier of the drawn yarn, at 0.85 to 1.15.

8. The process of claim 1 wherein the process is performed while maintaining the draw texturing speed at 75 to 600 m/min.

9. The process of claim 2 wherein the process is performed while maintaining the draw ratio at 2.2 to 2.8.

10. The process of claim 1 wherein the yarn is bent by at least 2 yarn guides provided between the false twister and the draw rollers, and the total sum of the bent angles is adjusted to from 30° to 270°.

11. The process of claim 10 wherein the process is controlled so that the yarn runs between the heat-treating heater and the false twister for 0.13 to 0.3 second in air at room temperature.

12. The process of claim 1 wherein the undrawn yarn is made to run from the inlet of the heat-treating heater to a point  $l$  mm apart from it while being preheated at 60° to 150°C. without contacting with the heated surface of the heater, and then the yarn is brought into contact with the heated surface of the heater,  $l$  above being defined by the following equations

$$l \geq 5$$

and

$$0.03x + 0.2y - 15l \leq 0.3x + 2y + 100$$

wherein  $x$  is the denier of the undrawn yarn and  $y$  is the speed of feeding the undrawn yarn (m/min.).

13. The process of claim 7 wherein the operation is started with a false twist multiplier 50 - 85 % of that in normal operation without bringing the yarn into contact with the heat-treating heater, and then the yarn is brought into contact with the heat-treating heater and the false twist multiplier is increased to a predetermined value.

14. The process of claim 8 wherein yarn stringing is performed by initiating the operation at a draw texturing speed expressed by the equation

$$5 \leq v \leq 80 - \left( \frac{De}{5} \right)$$

wherein  $V$  is the draw texturing speed, and  $De$  is the denier of the undrawn yarn, and then the draw texturing speed is increased to a predetermined value.

15. The process of claim 1 wherein at the time of initiating the operation, the yarn is strung up by keeping the undrawn yarn from the surface of the heat-treating heater so that it does not come close to it, and then draw texturing of the yarn is started while passing the yarn through a zone maintained at a temperature of 50°C. to 130°C. near the surface of the heat-treating heater, and thereafter, the yarn is brought into contact with the surface of the heat-treating heater.

16. The process of claim 1 wherein before an undrawn yarn package being processed becomes empty, the end of the undrawn yarn on the package is tied with the forward end of an undrawn yarn on an undrawn yarn package to be processed subsequently, after cold drawing each end of the undrawn yarns.

17. The process of claim 1 wherein the resulting draw textured yarn is additionally heat-treated at a temperature of 160°C. to 250°C. while allowing a shrinkage of 10 not more than 50 % or maintaining it at constant length.

\* \* \* \* \*

15

20

25

30

35

40

45

50

55

60

65